

# UNITED STATES PATENT OFFICE.

ALBERT L. CLAPP, OF DANVERS, MASSACHUSETTS.

## METHOD OF MAKING PAPER AND FIBER BOARD.

1,389,936.

Specification of Letters Patent. Patented Sept. 6, 1921.

No Drawing.

Application filed June 23, 1920. Serial No. 391,162.

To all whom it may concern:

Be it known that I, ALBERT L. CLAPP, a citizen of the United States, residing at Danvers, in the county of Essex and State 5 of Massachusetts, have invented new and useful Improvements in Methods of Making Paper and Fiber Board, of which the following is a specification.

This invention has relation to the manufacture 10 of a fibrous material which may be employed for the production of paper as fiber board or analogous products.

In the manufacture of beet sugar, a residual waste or pressed pulp remains, 15 which comprises fiber or cellular material, proteid, and other organic substances, and this pulp constitutes one of the essential ingredients or component raw materials employed in the process which I shall describe.

20 I have discovered that when beet pulp is digested in an aqueous solution of sodium carbonate, under heat and pressure, more or less of the proteid is dissolved, and may be precipitated by means of a suitable agent 25 such as aluminum sulfate, to constitute a size for fibrous materials. I have further found that if this digestion takes place in the presence of the fibrous material, the dissolved proteid will permeate the fibers of 30 such material, and may subsequently be precipitated therein and thereon.

As an example of my process, I may cite the following:

35 1000 parts by weight of cotton fiber, mechanical or chemical wood pulp or other suitable cellulosic material; 500 parts of pressed beet pulp; 50 parts of sodium carbonate; and sufficient water to cover the mass, are loaded into a digester, and the 40 cover thereof is closed. Steam is injected from time to time to cook the mass at about fifteen pounds pressure for about two hours, care being taken not to prolong the cooking sufficiently to injure the cellulose fibers of 45 the beet pulp. During this digestion certain proteid constituents of the beet pulp go into solution and are cooked into the cellulose fibers. Then the contents of the digester are withdrawn and delivered to a 50 beating engine, with additional water, if necessary, to insure a free circulation of the stock in the beater. The beating action is continued until the stock has been suffi-

ciently reduced and disintegrated, and then 55 aluminum sulfate is added and beaten into the mass to cause precipitation of the dissolved proteid in and on the fibers. The stock may now be formed into sheets by the aid of any suitable paper making or web forming machine. When the materials are 60 supplied to the digester in the proportions hereinbefore recited, I usually form the web in convolutions on the suction cylinder of a wet machine, until a sheet is formed, of a predetermined caliper, which is then slit, removed and dried, and, if desired, subjected to pressure. The sheet material thus produced is horny, hard and relatively inflexible,—presenting somewhat the appearance 65 of very hard fiber board. If desired, sodium 70 resinate may be supplied to the beater before the introduction of the aluminum sulfate, and the proportion of the latter increased to cause the precipitation of aluminum resinate 75 on the fibers and thus further size the stock.

If it is desired to produce a flexible web or sheet of paper, the proportion of beet pulp furnished to the digester should be 80 decreased.

What I claim is:—

1. A process which comprises digesting beet pulp with heat and pressure in the presence of an aqueous solution of sodium carbonate, to dissolve certain constituents thereof, and then precipitating the same with a precipitating agent. 85

2. A process which comprises digesting cellulosic material and beet pulp with heat and pressure in the presence of sodium carbonate, and then precipitating dissolved constituents of the beet pulp in and on the cellulose fibers. 90

3. A process which comprises digesting cotton fibers and beet pulp with heat and pressure in the presence of sodium carbonate, and then precipitating dissolved constituents of the beet pulp in and on the cotton fibers. 95

4. A process which comprises cooking cellulose fibers and beet pulp in a sodium carbonate solution under pressure in a closed digester, then subjecting the mass to a disintegrating operation, and then adding a precipitating agent to precipitate certain dissolved constituents of the beet pulp. 100

5. A process which comprises cooking cel-

105

lulose fibers and beet pulp in a sodium carbonate solution under pressure in a closed digester, then subjecting the mass to a dis-integrating operation, then adding a pre-  
cipitating agent to precipitate certain dis-  
solved constituents of the beet pulp, and  
finally forming the pulped mass into a sheet.

6. A fibrous material comprising cellulose

fibers and a sizing compound which is pre-  
cipitated from the soluble constituents of 10  
beet pulp digested with heat and pressure  
in the presence of sodium carbonate.

In testimony whereof I have affixed my  
signature.

ALBERT L. CLAPP.